



US007749344B2

(12) **United States Patent**  
**Sengupta**

(10) **Patent No.:** **US 7,749,344 B2**  
(45) **Date of Patent:** **Jul. 6, 2010**

(54) **HIGH PERFORMANCE, LOW TOXICITY HYPERGOLIC FUEL**

(75) Inventor: **Debasis Sengupta**, Madison, AL (US)

(73) Assignee: **CFO Research Corporation**,  
Huntsville, AL (US)

(\*) Notice: Subject to any disclaimer, the term of this patent is extended or adjusted under 35 U.S.C. 154(b) by 643 days.

(21) Appl. No.: **11/679,672**

(22) Filed: **Feb. 27, 2007**

(65) **Prior Publication Data**

US 2008/0202655 A1 Aug. 28, 2008

(51) **Int. Cl.**

**C06B 47/00** (2006.01)  
**C06B 31/00** (2006.01)  
**C06B 31/28** (2006.01)  
**C06B 47/04** (2006.01)  
**D03D 23/00** (2006.01)  
**D03D 43/00** (2006.01)

(52) **U.S. Cl.** ..... 149/1; 149/45; 149/46;  
149/74; 149/109.2; 149/109.4

(58) **Field of Classification Search** ..... 149/1,  
149/45, 46, 74, 109.2, 109.6  
See application file for complete search history.

(56) **References Cited**

**U.S. PATENT DOCUMENTS**

6,962,633 B1 \* 11/2005 McQuaid ..... 149/1

\* cited by examiner

*Primary Examiner*—Jerry Lorengo

*Assistant Examiner*—James E McDonough

(74) *Attorney, Agent, or Firm*—Tomas Friend

(57) **ABSTRACT**

Disclosed is a group of tertiary amine azides useful as hypergolic fuels for hypergolic bipropellant mixtures. The fuels provide higher density impulses than monomethyl hydrazine (MMH) but are less toxic and have lower vapor pressures than MMH. In addition, the fuels have shorter ignition delay times than dimethylaminoethylazide (DMAZ) and other potential reduced toxicity replacements for MMH.

**4 Claims, 2 Drawing Sheets**



FIG. 1



FIG. 2



FIG. 3



## HIGH PERFORMANCE, LOW TOXICITY HYPERGOLIC FUEL

### STATEMENT REGARDING FEDERALLY SPONSORED RESEARCH OR DEVELOPMENT

The U.S. Government may have certain rights in this invention pursuant to Contract No. W31PQ06C0167 awarded by the U.S. Army

### CROSS-REFERENCE TO RELATED APPLICATIONS

Not Applicable

### INCORPORATED-BY-REFERENCE OF MATERIAL SUBMITTED ON A COMPACT DISC

Not Applicable

### BACKGROUND OF THE INVENTION

#### 1. Field of the Invention

The present invention relates to a hypergolic rocket fuels that simultaneously possess high-performance propellant characteristics and low toxicity relative to Monomethylhydrazine (MMH). The fuels provide propellant performance as high as or higher than MMH, but have lower toxicity.

#### 2. Description of Related Art

Monomethylhydrazine (MMH) is a widely employed fuel in hypergolic, bipropellant systems. MMH possesses desirable propellant properties but it is highly toxic, carcinogenic, and corrosive. Although gelling has dramatically improved the safety of handling and storing the propellant, its toxicity and carcinogenicity are still of major concern. Therefore, there is a need for alternative liquid hypergolic fuels that are less carcinogenic and less toxic than MMH but also have equal or higher energy densities, lower vapor pressures and ignition delays than MMH. These fuels, like MMH, may be used in the form of gels to further improve safety.

Although DMAZ is hypergolic, its ignition delay with IRFNA is significantly longer than MMH. A longer ignition delay requires a larger combustion chamber to avoid pressure spikes that can damage the engine.

U.S. Pat. No. 6,013,143, incorporated by reference herein in its entirety, discloses three chemicals, each comprising a tertiary nitrogen and an azide functional group that are hypergolic when mixed with an oxidizer such as IRFNA, hydrogen peroxide, nitrogen tetroxide, and hydroxyl ammonium nitrate. The chemicals are dimethylaminoethylazide (DMAZ), pyrrolidineylethylazide (PYAZ), and bis (ethyl azide)methylamine (BAZ). Inhibited Red Fuming Nitric Acid (IRFNA) type IIIB and monomethyl hydrazine (MMH) deliver a specific impulse of 284 lb<sub>f</sub> sec/lb<sub>m</sub> and a density impulse of 13.36 lb<sub>f</sub> sec/cubic inch in a rocket engine operating a pressure of 2000 psi. DMAZ, PYAZ, and BAZ are proposed as potential replacements for MMH. DMAZ, under the same conditions as MMH, delivers a specific impulse of 287 lb<sub>f</sub> sec/lb<sub>m</sub> and a density impulse of 13.8 lb<sub>f</sub> sec/cubic inch. The patent discloses the mixing of the hypergolic fuel chemicals with gellants and additives such as aluminum and boron to increase specific impulse and density impulse values.

U.S. Pat. No. 6,926,633, incorporated by reference herein in its entirety, discloses a family of amine azides having cyclic structures and for use as hypergolic rocket propellants. The amine azide compounds comprise at least one amine, includ-

ing tertiary amines, and an azide functional group pendant from a cyclic structure. The propellants are disclosed as being used with oxidizers and, optionally with catalysts present in fuel or oxidizer. Fuel properties for the amine azides are provided based on computational quantum chemistry calculations.

U.S. Pat. No. 6,949,152, incorporated by reference herein in its entirety, discloses hypergolic propulsion systems comprising a fuel composition and an oxidizer composition. The fuel composition contains an azide compound having at least one tertiary nitrogen and at least one azide functional group. The oxidizer contains hydrogen peroxide in water. The hypergolic reaction between oxidizer and fuel is catalyzed by a transition metal, preferably compounds of cobalt and manganese.

Unlike hypergolic fuels disclosed previously, the present fuels exhibit lower toxicity and higher performance than MMH. The fuels require no catalyst to achieve high performance and are hypergolic with commonly used oxidizers.

The fuels of the present invention may be used alone, in combination with each other, or in combination with other fuels in blends.

### BRIEF SUMMARY OF THE INVENTION

The present invention is a group of tertiary amine azide chemicals useful as hypergolic fuels for hypergolic bipropellant mixtures. The fuels provide higher density impulses than MMH but are less toxic and have lower vapor pressures than MMH. In addition, the fuels have shorter ignition delay times than DMAZ and other potential reduced toxicity replacements for MMH.

### BRIEF DESCRIPTION OF THE SEVERAL VIEWS OF THE DRAWINGS

FIG. 1 illustrates the structures of chemicals (I)-(VIII).

FIG. 2 illustrates the structures of chemicals (IX)-(XI).

FIG. 3 illustrates the structures of chemicals (XII) and (XIII).

### DETAILED DESCRIPTION OF THE INVENTION

The present invention is a rocket fuel composition comprising one or more of the molecules shown in FIGS. 1-3. The fuel is hypergolic when combined with a strong oxidizer such as IRFNA, hydrogen peroxide, nitrogen tetroxide, or hydroxyl ammonium nitrate. Relevant chemical and physical properties of the molecules have been calculated using validated molecular modeling techniques, including quantum chemistry and Conductor-like Screening MOdel for Real Solvent (COSMO-RS) methods. The fuel molecules have been selected for one or more desirable propellant properties including:

High heat of formation: Heat of formation is directly related to the specific impulse which is a measure of energy content in the molecule.

Density: Density of the liquid fuel is important because density impulse, a measure of fuel performance, is the product of density and specific impulse.

Vapor Pressure: Low vapor pressure improves safety during handling and storage.

Absence of N—N single bonds: Absence of N—N single bonds reduces toxicity.

Short Ignition Delay: Short ignition delay time with the oxidizer is desirable to minimize engine size and damage resulting from pressure spikes during combustion.

## Heats of Formation

First-principle ab initio quantum chemistry methods are the most accurate and suitable technique for calculations of molecular geometries, heats of formations, and activation barriers. Quantum chemistry techniques are based on the principles of quantum mechanics. The procedure numerically solves a many-electron Schrödinger equation to obtain a molecular wave function and energy. The molecular energies can be used to calculate heats of formation.

CBS-QB3 [Ochterski, 1995; Montgomery, 2000] and PBEPBE/6-311++G(d,p) [Perdew, 1996] combined with isodesmonic reaction methods were used to calculate the heats of formations, and activation barriers for the molecules in FIGS. 1-3. Heat of vaporization was calculated using a COSMO-RS technique [Klamt, 1995 and 2000]. Table 1 shows the computed heats of formation for hydrazine, MMH, DMAZ, and the compounds of the present invention. Numbers in parentheses are National Institutes of Standards and Technology (NIST) experimental data. The molecules of the present invention possess higher heats of formation than MMH, and are therefore expected to possess specific impulse values that exceed those for MMH.

## Densities

Wong et al. [Wong, 1995] have developed a procedure for calculating molecular volume, defined as the volume occupied by 0.001 au (1 au=6.748 e/Å) electron density envelope. Once the molecular volume is known, the density can be computed using molecular weight. Calculated and known densities were compared for a number of amines and amine azides to validate density calculations.

Calculations were performed at the PBEPBE/6-311++G(d,p) level. Table 2 compares experimentally measured densities with calculated densities with and without corrective correlation. Error! Reference source not found, tabulates the predicted densities of molecules shown in FIGS. 1-3.

TABLE 1

| Molecule  | Computed Heats of Formation             |                                       |
|-----------|-----------------------------------------|---------------------------------------|
|           | Gas Phase $\Delta H_f^{298} K$ kcal/mol | Gas Phase $\Delta H_f^{298} K$ cal/gm |
| Hydrazine | 23.8 (22.8)                             | 744.9 (712.5)                         |
| MMH       | 23.0 (22.6)                             | 500.9 (492.2)                         |
| DMAZ      | 73.4                                    | 643.6                                 |
| I         | 96.2                                    | 858.9                                 |
| II        | 149.8                                   | 1361.9                                |
| III       | 110.1                                   | 781.0                                 |
| IV        | 134.8                                   | 1078.2                                |
| V         | 112.2                                   | 738.3                                 |
| VI        | 90.0                                    | 489.0                                 |
| VII       | 112.2                                   | 679.7                                 |
| VIII      | 110.0                                   | 516.3                                 |
| IX        | 114.3                                   | 747.2                                 |
| X         | 89.6                                    | 577.8                                 |
| XI        | 128.5                                   | 537.6                                 |
| XII       | 106.5                                   | 578.9                                 |
| XIII      | 144.6                                   | 510.9                                 |

TABLE 2

| Molecule                   | Calculated and Measured Densities |                      |                           |
|----------------------------|-----------------------------------|----------------------|---------------------------|
|                            | Computed Density (raw data)       | Experimental density | Density after correlation |
| $(\text{CH}_3)_2\text{NH}$ | 0.9307                            | 0.671                | 0.7038                    |
| $\text{CH}_3\text{NH}_2$   | 0.9140                            | 0.694                | 0.6849                    |
| $\text{CH}_3\text{N}_3$    | 1.1225                            | 0.869                | 0.9212                    |

TABLE 2-continued

| Molecule                                      | Calculated and Measured Densities |                      |                           |
|-----------------------------------------------|-----------------------------------|----------------------|---------------------------|
|                                               | Computed Density (raw data)       | Experimental density | Density after correlation |
| $\text{C}_2\text{H}_5\text{N}_3$              | 1.1187                            | 0.876                | 0.9170                    |
| 2-azido-N-cyclopropylethanamine               | 1.1649                            | 0.990                | 0.9693                    |
| $\text{H}_2\text{NCH}_2\text{CH}_2\text{N}_3$ | 1.1791                            | 1.040                | 0.9855                    |
| I, DMAZ                                       | 1.1100                            | 0.933                | 0.9096                    |
| $\text{HN}_3$                                 | 1.3116                            | 1.090                | 1.1356                    |

TABLE 3

| Molecule | Predicted Densities |                                     |
|----------|---------------------|-------------------------------------|
|          | Density (raw data)  | Density after using the correlation |
| I        | 1.1320              | 0.9346                              |
| II       | 1.1334              | 0.9362                              |
| III      | 1.2114              | 1.0246                              |
| IV       | 1.3325              | 1.1619                              |
| V        | 1.4048              | 1.2438                              |
| VI       | 1.2153              | 1.0290                              |
| VII      | 1.3801              | 1.2158                              |
| VIII     | 1.2347              | 1.0510                              |
| IX       | 1.2449              | 1.0626                              |
| X        | 1.1381              | 0.9415                              |
| XI       | 1.3249              | 1.1532                              |
| XII      | 1.2433              | 1.0608                              |
| XIII     | 1.2539              | 1.0728                              |

Specific and density impulse are the two most important parameters describing the performance of a fuel. Density impulse is a measure of the performance per volume of the fuel. Table 4 shows the computed specific and density impulse for each of the molecules shown in FIGS. 1-3 with IRFNA as the oxidizer.

TABLE 4

| Molecule | Computed Specific and Density Impulse            |                                                                                        |                        |
|----------|--------------------------------------------------|----------------------------------------------------------------------------------------|------------------------|
|          | $I_{sp}$ (lb <sub>f</sub> ·sec/lb <sub>m</sub> ) | Density Impulse = density * $I_{sp} * 10^{-3}$ (lb <sub>f</sub> ·sec/ft <sup>3</sup> ) | % Improvement over MMH |
| I        | 280.0                                            | 16.3                                                                                   | 4.1                    |
| II       | 286.4                                            | 16.7                                                                                   | 6.6                    |
| III      | 280.2                                            | 17.9                                                                                   | 14.2                   |
| IV       | 280.7                                            | 20.4                                                                                   | 29.7                   |
| V        | 272.4                                            | 21.2                                                                                   | 34.7                   |
| VI       | 276.8                                            | 17.8                                                                                   | 13.3                   |
| VII      | 267.8                                            | 20.3                                                                                   | 29.5                   |
| VIII     | 278.0                                            | 18.2                                                                                   | 16.2                   |
| IX       | 283.4                                            | 18.8                                                                                   | 19.7                   |
| X        | 277.5                                            | 16.3                                                                                   | 3.9                    |
| XI       | 277.6                                            | 20.0                                                                                   | 27.3                   |
| XII      | 279.0                                            | 18.5                                                                                   | 17.7                   |
| XIII     | 278.4                                            | 18.6                                                                                   | 18.8                   |

The  $I_{sp}$  values were calculated using the PROPER thermochemical code and correspond to the optimum fuel/IRFNA ratio. Table 4 shows that there is a substantial improvement of density impulse over MMH.

## Synthesis of Hypergolic Fuels

The molecules of the present invention may be synthesized by those skilled in the art using known chemical synthetic reactions. For example, the synthesis of compound V can be accomplished by the using the known condensation of guanidines with haloacetates [Webb, 2003] followed by reac-

## 5

tion with  $\text{PCl}_5$  and treatment with  $\text{NaN}_3$ . Compound VII can be prepared from 2,4-dichlorotriazine by sequential substitution of the chlorine atoms. The dichloride 5 can be prepared by condensation [Harris, 1981] of iminyl chloride. The preparation of compound XII can be accomplished, for example, by transamination [Flores-Parra, 1999] between two symmetric triazinanes.

## REFERENCES

- The following references are incorporated by reference in their entirety.
- Flores-Parra, A.; Sanchez-Ruiz, S. A. *Heterocycles* (1999) 51: 2079-2092.
- Godbout, N, Salahub, D. R., Andzelm, J., and Wimmer, E.; *Can. J. Chem.* (1992) 70: 560
- Harris, R. L. N. "The synthesis of Triazines from N-Cyano-carbamimidates" *Synthesis* (1981) 1981:907-908
- Klamt, A; *J. Phys. Chem.*, (1995) 99: 222
- Klamt A.; *Fluid Phase Equil.*, (2000) 172: 43
- McQuaid, M. J.; Stevenson, W. H., and Thompson; D. M. (2004) 24th Army Science Conference, Orlando, Fla.
- Montgomery Jr. J. A., Frisch, M. J. Ochterski, J. W., and Petersson, G. A. (2000) *J. Chem. Phys.* 112: 6532.
- Ochterski, J. W., Petersson, G. A., and Wiberg, K. B. (1995) *J. Am. Chem. Soc.* 117: 11299

## 6

- Perdew, J. P., Burke, K., and Ernzerhof, M. (1996) *Phys. Rev. Lett.* 77, 3865
- Wong, M. W., Wiberg, K. B., Frisch, M. J. (1995) *J. Camp. Chem.* 16:385

5 What is claimed is:

10 1. A hypergolic bipropellant combination comprising an oxidizer and a fuel, wherein the fuel comprises an amine azide chemical having the structure  $(\text{CH}_3)_2\text{N}-\text{R}_1$ , and wherein  $\text{R}_1$  is



2. The hypergolic bipropellant combination of claim 1 further comprising a gellant mixed with the fuel or oxidizer.

3. The hypergolic bipropellant combination of claim 1 wherein the oxidizer is selected from IRFNA, hydrogen peroxide, nitrogen tetroxide, and hydroxyl ammonium nitrate.

20 4. The hypergolic bipropellant combination of claim 1 wherein the fuel is a mixture comprising the amino azide chemical as an additive.

\* \* \* \* \*

UNITED STATES PATENT AND TRADEMARK OFFICE  
**CERTIFICATE OF CORRECTION**

PATENT NO. : 7,749,344 B2  
APPLICATION NO. : 11/679672  
DATED : July 6, 2010  
INVENTOR(S) : Sengupta

Page 1 of 1

It is certified that error appears in the above-identified patent and that said Letters Patent is hereby corrected as shown below:

**Title Page, item 73, Assignee**

Delete "CFO" and insert -- CFD --, therefore.

**In the Specification, Column 1**

In Column 1, Lines 7-9, delete "The U.S. Government may have certain rights in this invention pursuant to Contract No. W31PQ06C0167 awarded by the U.S. Army" and insert -- This invention was made with Government support under contract W31P4Q-06-C-0167 awarded by the US Army. The Government has certain rights in this invention. --, therefore.

Signed and Sealed this  
Ninth Day of April, 2013



Teresa Stanek Rea  
*Acting Director of the United States Patent and Trademark Office*